

Dec. 9, 1924.

1,518,638

H. DE OLANETA

DRY CELL

Original Filed Dec. 22, 1919



Inventor

Harold de Olaneta

By

Alfred P. Deacon

Attorney

## UNITED STATES PATENT OFFICE.

HAROLD DE OLANETA, OF NEW HAVEN, CONNECTICUT, ASSIGNOR TO WINCHESTER REPEATING ARMS COMPANY, OF NEW HAVEN, CONNECTICUT, A CORPORATION OF CONNECTICUT.

## DRY CELL.

Original application filed December 22, 1919, Serial No. 346,694. Divided and this application filed May 3, 1920. Serial No. 378,457.

*To all whom it may concern:*

Be it known that I, HAROLD DE OLANETA, of New Haven, county of New Haven, State of Connecticut, have invented certain new 5 and useful Improvements in Dry Cells, of which the following is a full, clear, and exact description.

This invention relates to galvanic cells and more particularly to dry cells.

10 The present application is a division of my application, Serial No. 346,694, filed December 22nd, 1919, and pertains more especially to the paste employed in the cell.

In dry cells of the type now found on the 15 market in large numbers, and especially those used for pocket flash lights or hand lamps, the zinc electrode is in the form of a cup in which are contained a carbon electrode with a surrounding body of depolarizing material, and an exciting paste interposed between the depolarizing material and the side wall of the cup. The depolarizing material usually consists of a mixture of manganese dioxid and carbon 20 which is formed into a block or cartridge about the carbon electrode and is contained within an envelope or bag of cheese cloth or the like.

In the manufacture of cells of this type, 25 the paste when placed in the cell ordinarily contains a solution of sal ammoniac, which is the principal exciting agent, and a solution of zinc chlorid, which, owing to its deliquescent nature, serves to keep the 30 paste moist. The depolarizing mixture, consisting of finely divided manganese dioxid and carbon (graphite), is usually moistened with a solution containing ammonium chlorid and zinc chlorid, so as to facilitate 35 the passage of the ions from one electrode to the other through the depolarizing body and paste.

Cells made up in the usual way, with 40 an ammonium-chlorid-containing paste in direct contact with the zinc, are apt to deteriorate considerably before they are placed in use, owing to the fact that, due to local action, the ammonium chlorid commences its 45 attack on the zinc as soon as the parts of the cell are put together. Local action is

set up, for example, as a result of the presence of impurities in the zinc, or by reason of differences in the molecular structure of the same at different parts of the cup. Under present conditions of manufacture and distribution, there is usually a considerable interval between the time when the cell is first assembled and the time when it reaches the consumer for use. It is not uncommon for the cells to remain in the 55 factory a week or longer, owing to delays in packing and shipping. Furthermore, when they leave the factory it takes some time for them to reach the retailer, and, of course, they may remain on the shelf of 60 the retailer for a long period before they are purchased and used. Consequently when a cell is finally put into use, the zinc cup is likely to be considerably eaten away, 65 and the active life of the cell is, therefore, 70 seriously impaired.

One of the primary objects of my invention is to eliminate the above mentioned drawback as far as possible. I provide a 75 cell in which the action of the sal ammoniac on the zinc while the cell is being shipped and while it is on the shelf is avoided to a large extent. The cell of my invention does not have maximum efficiency when first assembled, but it reaches maximum efficiency 80 some time thereafter, in other words, at about the time that it comes into the hands of the user. In this manner the life of the cell in the hands of the user is considerably increased.

Another object of my invention is to 85 simplify and improve the process of manufacturing dry cells of the type indicated. In ordinary methods of manufacture, there are numerous drawbacks and inconveniences 90 arising out of the incorporation of the sal ammoniac and zinc chlorid in the same body, more particularly in the paste. For example, there are difficulties as regards the proper proportioning of the two solutions 95 which are commonly employed. Again, the sal ammoniac-containing paste is difficult to handle in the factory owing to the fact that sal ammoniac is a climbing salt. One of the greatest objections, however, is that 100

when sal ammoniac is incorporated in the paste before the latter is placed in the cell, the paste will not keep for any length of time. It has to be used immediately after being mixed up, as otherwise there is apt to be a formation of mold.

Another object, therefore, of my present invention is to overcome these difficulties and disadvantages incident to the manufacture of the cells.

To these and other ends, the invention consists in the novel features to be herein-after set forth and claimed.

The accompanying drawing shows in vertical, central section a dry cell made in accordance with the invention.

The cell comprises the usual zinc cup 1 constituting the positive electrode. The negative carbon electrode 2 has tamped about the same a block or cartridge 3 of suitable depolarizing material; and interposed between the side wall of the cup and the depolarizing material is a paste 4. The depolarizing cartridge is usually contained 20 in a bag or envelope 5 of cheese cloth or the like. It is centered in the cup at the bottom by a suitable centering washer 6. At the top of the cell the latter is sealed in any suitable manner, as by a pitch seal 7 on top of a paper washer 8. The carbon electrode is provided with the usual contact cap 9.

In carrying out my invention, I provide a paste which is initially devoid of sal ammoniac. The paste is preferably composed of wheat flour or some other cereal, zinc chlorid solution, and a mercury compound. In making up a batch of paste for the manufacture of a number of cells, I mix together, for example, 12.5 kilograms of wheat flour, 50 litres of zinc chlorid solution at 27° Baumé, and 12.5 grams of mercuric chlorid. The ingredients are mixed together until all of the flour is dissolved, and the mass is stirred, while being cooked, until a stiff paste is formed. The cooking is effected before the paste is placed in the cell.

The depolarizing body preferably comprises a mixture of manganese dioxid, graphite, and sal ammoniac, for example, in the proportions of 37.5 units of manganese hydrate, 12.5 units of graphite and 10 units of sal ammoniac. These ingredients, which are in a fine state of subdivision, are mixed with water until the mass is plastic and homogeneous, whereupon it is formed into the block or cartridge 3 about the carbon electrode 2 in a manner well understood in the art.

60 The paste will keep for a long time and does not have to be used at once owing to the fact that the zinc chlorid is of an anti-septic nature and acts as a preservative for the vegetable substance, e. g. wheat flour.

The drawbacks incident to the incorporation in the paste of ammonium chlorid, which tends to create a bacterial food, are eliminated.

When the cell is first put together, the ammonium chlorid does not immediately commence its attack on the zinc, owing to the fact that it must first traverse the paste. The sal ammoniac passes out only gradually from the cartridge into the paste and to the zinc. Thus the cell is not at maximum efficiency when first assembled, as is ordinarily the case, but reaches maximum efficiency after a definite interval has passed, depending upon the distance between the depolarizing cartridge and the side wall of the zinc cup. For example, with the smaller sizes of cells commonly used for pocket flash lights, the distance which has to be traversed by the sal ammoniac before it reaches the zinc, is such that maximum efficiency is not obtained for a period varying from two weeks to a month. In a larger size, where the sal ammoniac has to traverse a greater distance, the conditions usually obtaining in a freshly made cell do not obtain for approximately three months. Therefore there is likelihood that the cell will not reach its maximum efficiency until about the time that it is placed in use. At any rate the life of the cell in the hands of the consumer is considerably increased owing to the fact that the length of time that the sal ammoniac acts on the zinc previous to the use of the cell, is considerably reduced.

In the case under discussion, the sal ammoniac passes outward through the porous envelope 5 of the cartridge into the paste and to the zinc, and the zinc chlorid in the paste passes into the cartridge; but it will be apparent that the invention is not limited to a cell wherein the depolarizing cartridge has a porous envelope. Regardless of whether or not an envelope is employed, the paste takes up sal ammoniac from the cartridge and the cartridge takes up zinc chlorid from the paste. Furthermore, these substances are distributed as needed for the best working of the cell. Heretofore, in manufacturing cells wherein the paste contained both zinc chlorid and ammonium chlorid, there was considerable difficulty in properly proportioning these two substances. It was necessary to weigh the substances and to compare the density of their solutions, etc., and even where great care was exercised in compounding the paste, the results were not always satisfactory. In the present case, however, the process of manufacture is considerably simplified, because it is not necessary to mix the chlorids and because such great care in attempting to reach a definite proportion of the ingredients is unnecessary. With my improved

cell, the ammonium chlorid is fed or supplied to and taken up by the paste in the proper quantity for the best working, and the zinc chlorid is fed to and taken up by the cartridge in the proper quantity for best working, regardless of the quantities of those substances which are used, within certain limits.

The chlorid of mercury in the paste serves the usual purpose of amalgamating the zinc.

So far as manufacturing advantages are concerned, it will be understood that a paste made in the manner herein described, which is devoid of ammonium chlorid when first compounded, will keep better and is much easier to handle than a paste in which ammonium chlorid is incorporated. The ammonium chlorid not only starts the forming of mould, but climbs out of the paste and over the containing vessels and utensils employed in the storage and handling of the paste, thus causing much inconvenience. Owing to these drawbacks, and the tendency of the sal ammoniac to dry up the paste, it has been impossible heretofore to use paste prepared any considerable length of time in advance of the time when it was placed in the zinc cups, and there was, therefore, considerable waste.

While my improved cell ordinarily does not reach its maximum efficiency until some time after it has left the factory, it can be readily brought to maximum efficiency by placing it in a closed circuit. When the cell is used for lighting a small lamp, for example, the passage of electric current through the cell has the effect of hastening the passage of the electrolyte, viz., the sal ammoniac, to the zinc. Of course, the zinc chlorid in the paste serves as an electrolyte to a sufficient extent to establish a current through the cell when the circuit is closed, and such current has the effect of drawing out the sal ammoniac from the depolarizing body so that the former will quickly reach and act on the zinc for the establishment of a strong current. While, therefore, cells made in accordance with the present invention meet the present conditions of slow distribution to the consumer, this advantage is not coupled with any appreciable lack of efficiency in the cell as freshly assembled.

The mercuric chlorid used in the paste as an amalgamator is of an antiseptic or preservative character, as well as the zinc chlorid, and hence all of the materials added to the wheat flour or the like tend to preserve the same and arrest decomposition.

While I have referred herein to sal ammoniac as being the principal exciting agent and to zinc chlorid as a paste moistening agent having a certain electrolyte value, it is to be understood, of course, that I do not limit myself in all aspects of the invention

to the use of these particular salts, or, in fact, to the employment of two distinct salts.

Various changes may be made in the details of the procedure and in the composition and arrangement of parts as herein described, without departing from the scope of my invention as set forth in the claims.

What I claim is:

1. In a dry cell, a paste containing cereal, an amalgamator and an electrolyte, the electrolyte content when the paste is fresh consisting substantially entirely of a salt material of a preservative character, said paste being designed to receive and distribute an excitant placed in juxtaposition thereto.

2. In a dry cell, a stiff paste containing cereal, an amalgamator and an electrolyte, said electrolyte consisting substantially entirely of a salt material which preserves the cereal against mold, and said paste being designed to receive and distribute an excitant placed in juxtaposition thereto.

3. In a dry cell having a zinc cup and a depolarizing cartridge, a stiff, precooked paste interposed between said parts and containing cereal and an electrolyte, substantially the whole electrolyte content being mold preventing, but said paste being adapted to absorb and distribute another electrolyte placed in juxtaposition thereto in the cell.

4. A paste for use in dry cells, containing wheat flour, zinc chlorid solution and mercuric chlorid in approximately the proportions of 12.5 kilograms of flour, 50 litres of zinc chlorid solution at 27 Baumé, and 12.5 grams of mercuric chlorid.

5. A paste for use in dry cells, comprising a stiff cooked mass consisting of wheat flour, zinc chlorid solution and mercuric chlorid.

6. In a dry cell, a paste cooked before the same is placed in the cell and comprising a stiff mass of cereal, chlorid solution and mercury compound mixed together before cooking, said paste being adapted to receive and distribute an excitant placed in juxtaposition thereto.

7. A stiff, precooked paste for dry cells, containing vegetable matter and an electrolyte, substantially the whole electrolyte content consisting of an antiseptic deliquescent salt solution, said paste being adapted to receive and distribute an excitant placed in juxtaposition thereto.

8. A stiff, precooked paste for dry cells, of electrolytic character, which, when fresh, is substantially devoid of ammonium chlorid and other mold forming matter, said paste being adapted to receive and distribute an excitant placed in juxtaposition thereto.

9. A stiff paste for dry cells, containing cereal and an electrolytic content practically devoid of ammonium chlorid, said paste be-

ing of a character such that it will receive and distribute quite slowly an ammonium chlorid solution placed in juxtaposition thereto.

5. 10. A stiff paste for dry cells, cooked before the same is placed in the cell, and comprising a cereal and a weak electrolyte solution mixed together before cooking, but sub-

stantially devoid of any material forming or tending to form with the cereal bacterial food, and said paste being adapted to receive and slowly distribute an excitant placed in juxtaposition thereto. <sup>10</sup>

In witness whereof, I have hereunto set my hand on the 30th day of April, 1920.

HAROLD DE OLANETA.